

## UNITED STATES PATENT OFFICE

2,690,426

## LUBRICATING COMPOSITIONS

George D. Jefferson, Embreeville, Pa., and Richard De Mott Fine III, Merchantville, N. J., assignors to Atlas Powder Company, Wilmington, Del., a corporation of Delaware

No Drawing. Application March 7, 1950,  
Serial No. 148,258

19 Claims. (Cl. 252—8.8)

1

The present invention relates to a novel composition of matter.

The object of the invention is to provide compositions of matter of low volatility, high emulsifiability and high lubricity.

Such compositions of matter are useful as textile lubricants, cutting oils, flushing oils, etc., and generally wherever an emulsifiable lubricant is desired.

The textile arts in particular find necessary the use of a treating agent which upon application will lubricate, not evaporate during storage of the textile and which may be removed by simple scouring. The various steps of forming and handling yarns of cotton, wool, viscose, nylon, cellulose acetate, etc., are high speed operations requiring the reduction of internal and external friction by treatment of the filaments, threads, fibers and the like. The lubricant must not be so volatile that it is lost to an effective extent from the fibers should they be placed in storage between steps. Furthermore, it is frequently necessary that such lubricants be removed prior to after operations such as dyeing, hence the necessity for ease of removal. Lastly, the consistency of the lubricant should be such as to adapt itself to conventional modes of application and not require solvents, heating, etc.

The prior art has extensively employed mineral oils as textile lubricants. As employed in the past either alone or modified, these oils have been objectionable due to their high volatility and poor scourability properties. Thus, difficulty in oil removal frequently has interfered with dyeing and other after treatments. Furthermore, upon storage of the textile, evaporation of these oils leaves the material harsh and unsuitable for textile manufacture.

There are less volatile non-mineral oil lubricants that are very effective in their lubricity when applied to textile treating purposes. These are objectionable, however, due to low scourability, high cost and high viscosity. This latter difficulty necessitates special modes of application, rendering such treatment processes still more costly.

It has been discovered that blends of mineral oil lubricants and certain non-mineral oil type lubricants may be obtained which in combination with a mineral oil soluble dispersing agent combine the very desirable properties of high lubricity, low volatility, excellent scourability and suitable viscosity for direct application by conventional means.

Broadly, these desirable properties are attrib-

2

utable to novel compositions containing (1) from 51 to 98% refined mineral oil and (2) from 49 to 2% of a mixture containing (a) from 50 to 20% of a non-mineral lubricating compound of the structure:



wherein R is the residue formed by removal of active hydrogen from a compound of the class 10 consisting of aliphatic alcohols, acids, amines and amides containing from 12 to 18 carbon atoms solely substituted by hydrogen and R<sub>1</sub> is a member of the class consisting of hydroxyl, and residues of the class in the definition of R, x representing a number from 0 to 9 and y being an integer less than 3, and (b) from 50 to 80% of a suitable mineral oil soluble dispersing agent.

The preferred composition of matter contains 15 from 75 to 98% of the mineral oil, from 1 to 20 12.5% of the lubricating compound and from 1 to 20% of the mineral oil soluble dispersing agent.

The mineral oils employed as the base in this 20 composition are of the conventional, petroleum base, lubricating grade. Their viscosity may 25 vary through wide ranges depending upon the anticipated application. A particularly suitable oil for textile treatment is a refined, white mineral oil having a viscosity of 50 seconds Saybolt at 100° F. Such oils are available commercially from major oil companies and textile supply houses.

The non-mineral oil lubricant compound of the 30 class defined is typified by:

- 35 Polyoxyethylene ether of lauryl alcohol containing 2 oxyethylene groups
- 35 Polyoxyethylene ether of cetyl alcohol containing 10 oxyethylene groups
- 40 Polyoxyethylene stearic acid containing 3 oxyethylene groups
- 40 Polyoxyethylene palmitic acid containing 7 oxyethylene groups
- 45 Polyoxyethylene stearyl amine containing 4 oxyethylene groups
- 45 Polyoxyethylene stearyl amine containing 10 oxyethylene groups
- 50 Polyoxyethylene lauryl amine containing 1 oxyethylene group
- 50 Polyoxyethylene stearoyl amide containing 5 oxyethylene groups
- 50 Polyoxyethylene lauroyl amide containing 10 oxyethylene groups

These products, in the generally commercially available forms used, are mixtures of closely related compounds. Also blends of various species

of these lubricants can be made to obtain particular advantages in consistency, lubricity, and yarn softness.

It is understood, of course, that within the class of examples cited supra, there may exist oxyethylene substitution upon more than one reactive hydrogen where such is available, as for instance in the amino and amido derivatives. Also similar or dissimilar amido, amino and carboxy long chain residues may be substituted upon each end of the oxyethylene chain to produce such derivatives as the diester of polyoxyethylene glycol (Example 10 below).

The dispersing agent must be oil soluble. It serves the double function of rendering the mineral oil and non-mineral oil phases compatible as well as producing stability in the aqueous emulsions of the mixture. Suitable substances are the esters of fatty acids with aliphatic polyhydroxy compounds. The term "aliphatic" as employed in the specification and claims to describe this component is intended to include the inner ethers of polyhydroxy compounds such as the hexitans. Particularly valuable agents of this type may be formed by the reaction of acids such as myristic, stearic, palmitic, lauric and oleic with polyhydroxy compounds such as glycol, polyglycols, glycerol, polyglycerols, erythritol, pentaerythritol, the hexitans and hexitols and with ethylene oxide to form partial esters of polyoxyethylene ethers and polyoxyethylene ethers of partial esters. Preferred among these are the polyoxyethylene ethers of hexitan partial esters of fatty acids having from 12 to 18 carbon atoms wherein the ratio of oxyethylene groups to fatty acid radicals is from 3 to 8, and partial esters of fatty acids having from 12 to 18 carbon atoms with polyoxyethylene ethers of hexitols wherein the ratio of oxyethylene groups to fatty acid radicals is from 3 to 8.

The mineral oil soluble dispersing agent of the class defined is typified by:

Polyoxyethylene sorbitan monostearate containing 4 oxyethylene groups per mol

Polyoxyethylene sorbitan monooleate containing 5 oxyethylene groups per mol

Polyoxyethylene mannitan monolaurate containing 3 oxyethylene groups per mol

Polyoxyethylene sorbitan tristearate containing 20 oxyethylene groups per mol

Polyoxyethylene sorbitan trioleate containing 20 oxyethylene groups per mol

Polyoxyethylene sorbitan tripalmitate containing 16 oxyethylene groups per mol

Tetra-oleate of polyoxyethylene sorbitol containing 30 oxyethylene groups per mol

Mono-laurate of polyoxyethylene sorbitol containing 3 oxyethylene groups per mol

Mono-palmitate of polyoxyethylene sorbitol containing 6 oxyethylene groups per mol

The commercially available forms of these dispersing agents are eminently suited for use in this invention. They contain a mixture of specific compounds of the indicated types differing within a relatively narrow range in polyoxyethylene content, fatty acid (due to use of commercial fatty acid mixtures), and molecular structure (due to isomerism). Furthermore, different members of the class can be blended together to obtain desirable properties with respect to consistency and dispersing power.

The compositions according to the invention are produced by simple mixing of the components preferably accompanied by warming. The lubricants are not soluble in the mineral oil by themselves but are carried into solution or fine suspension by the oil soluble dispersing agents. In the case of certain concentrations some of the mixtures may be slightly hazy when formed. This haziness does not impair the usefulness of the compositions although clear apparent solutions are preferable where the material must undergo prolonged storage. In many cases the addition of a very small quantity of water to a hazy dispersion results in clearing it.

These compositions have low viscosities comparable to those of the mineral oil used and they may be applied to textile materials by the same means and with standard equipment used for mineral oil application. Evaporation of the mineral oil does not leave the textile material unlubricated because the polyoxyethylene lubricant is essentially non-volatile and is a much more efficient lubricant on a weight basis than the mineral oil. In addition, the polyoxyethylene lubricant has a pronounced softening effect, particularly on viscose yarn, that is unobtainable with mineral oil. The composition including the mineral oil is readily removable from the textile materials by simple scouring.

Many of the compositions of the invention are self-emulsifiable in water and may if desired be applied to the textile material in emulsion form. Whether emulsified or used in non-aqueous condition, the compositions can be applied by spraying, roller, dipping, or other conventional method.

The following examples illustrate typical conditioning agents according to the invention. The mineral oil used was a refined white 50w textile oil. The oil was warmed to about 60° C., the dispersing agent and lubricant were prewarmed and added with stirring.

| Example | Percent<br>Mineral<br>Oil | Dispersing Agent                                               | Percent | Lubricant                                                | Percent |
|---------|---------------------------|----------------------------------------------------------------|---------|----------------------------------------------------------|---------|
| 1.....  | 95                        | polyoxyethylene sorbitan monooleate-5 oxyethylene groups.      | 2.5     | polyoxyethylene stearyl alcohol<br>3 oxyethylene groups. | 2.5     |
| 2.....  | 80                        | same.....                                                      | 15.0    | polyoxyethylene stearyl alcohol<br>5 oxyethylene groups. | 5.0     |
| 3.....  | 80                        | same.....                                                      | 15.0    | polyoxyethylene stearic acid 7<br>oxyethylene groups.    | 5.0     |
| 4.....  | 95                        | same.....                                                      | 2.5     | polyoxyethylene stearyl amine<br>4 oxyethylene groups.   | 2.5     |
| 5.....  | 95                        | polyoxyethylene sorbitan tripalmitate-16 oxyethylene groups.   | 2.5     | polyoxyethylene stearoyl amide<br>5 oxyethylene groups.  | 2.5     |
| 6.....  | 75                        | tetraoleate of polyoxyethylene sorbitol-30 oxyethylene groups. | 15.0    | polyoxyethylene oleic acid-2-oxy-<br>ethylene groups.    | 10.0    |
| 7.....  | 60                        | polyoxyethylene sorbitan trioleate 20 oxyethylene groups.      | 25.0    | polyoxyethylene lauryl amine-<br>3 oxyethylene groups.   | 15.0    |

Tetra-laurate of polyoxyethylene mannitol containing 25 oxyethylene groups per mol

The following examples illustrates typical applications of the conditioning agents of the in-

vention. They also show a number of additional compositions of the type contemplated.

*Example 8*

Twenty denier twisted nylon yarn which had been previously sized with borated polyvinyl alcohol was treated in the coning process by passing over a roll turning in a trough of a conditioning agent having the following composition:

|                                                                   | Per cent |
|-------------------------------------------------------------------|----------|
| Polyoxyethylene stearic acid 3 oxyethylene groups                 | 2.5      |
| Polyoxyethylene ether of sorbitan monooleate-5 oxyethylene groups | 2.5      |
| White mineral oil (50w)                                           | 95.0     |

The yarn treated in this manner was found to produce superior knitting results when run on a full fashioned knitting machine and the conditioning composition was easily removed by scouring with the customary agents used for this purpose. Normal dyeing performance was noted.

*Example 9*

A dyed cotton knitting yarn was treated in the coning operation by passing over a roll turning in a trough containing a 20% emulsion in water of the conditioning agent of Example 2.

The yarn treated in this manner was found to produce superior knitting results when run on a tubular type knitting machine and the hand of the resulting fabric was very satisfactory.

*Example 10*

Scoured wool was treated by spraying with a conditioning agent having the following composition:

|                                                                   | Per cent |
|-------------------------------------------------------------------|----------|
| Polyoxyethylene stearic acid stearate 10 oxyethylene groups       | 10       |
| Polyoxyethylene ether of mannitan monooleate-5 oxyethylene groups | 10       |
| White mineral oil (50w)                                           | 80       |

The wool stock treated in this manner carded very well and the spinning characteristics were satisfactory.

*Example 11*

Scoured wool stock was treated as in Example 10 with a 20% emulsion in water of a conditioning agent having the following composition:

|                                                                   | Per cent |
|-------------------------------------------------------------------|----------|
| Polyoxyethylene stearyl amine 10 oxyethylene groups               | 5        |
| Polyoxyethylene ether of sorbitan monooleate-5 oxyethylene groups | 15       |
| White mineral oil (50w)                                           | 80       |

The subsequent processing of this treated wool stock showed excellent performance.

*Example 12*

Cellulose acetate was treated as it was being extruded or "spun" by the application of a conditioning agent having the following composition:

|                                                                   | Per cent |
|-------------------------------------------------------------------|----------|
| Polyoxyethylene oleic acid 9 oxyethylene groups                   | 10       |
| Polyoxyethylene ether of sorbitan monooleate-5 oxyethylene groups | 10       |
| White mineral oil (50w)                                           | 80       |

The application of the conditioning agent was so regulated that an amount equivalent to ap-

proximately 0.5% of the weight of the yarn was applied.

The yarn treated in this manner had a soft "hand" or feel and produced less static than untreated yarn when processed. The physical properties of this yarn were satisfactory.

*Example 13*

Freshly spun or "green" cakes of viscose rayon yarn which had been previously desulfurized, bleached and scoured, were treated on a cake processing machine with a 1% emulsion in water of a conditioning agent having the following composition:

|                                                                   | Per cent |
|-------------------------------------------------------------------|----------|
| Polyoxyethylene stearic acid 7 oxyethylene groups                 | 10       |
| Polyoxyethylene ether of sorbitan monooleate-4 oxyethylene groups | 10       |
| White mineral oil (50w)                                           | 89       |

The yarn treated in this manner and subsequently extracted and dried was found to be soft and to perform well in coning and all other operations. The physical properties of this yarn were satisfactory.

What is claimed is:

1. A composition comprising (1) from 51 to 98% of a refined mineral oil and (2) from 49 to 2% of a mixture containing (a) from 50 to 20% of a compound of the formula:



wherein R is the residue formed by removal of active hydrogen from a compound of the class consisting of aliphatic alcohols, acids, amines and amides containing from 12 to 18 carbon atoms solely substituted by hydrogen and R<sub>1</sub> is a member of the class consisting of hydroxyl and the residue formed by the removal of active hydrogen from a compound of the class consisting of aliphatic acids and alcohols containing 12 to 18 carbon atoms, solely substituted by hydrogen, x representing a number from 0 to 9 and y being an integer less than 3 and (b) from 50 to 80% of a mineral oil soluble material selected from the group consisting of polyoxyethylene ethers of hexitan partial esters of fatty acids having from 12 to 18 carbon atoms wherein the ratio of oxyethylene groups to fatty acid radicals is from 3 to 8, and partial esters of fatty acids having from 12 to 18 carbon atoms with polyoxyethylene ethers of hexitols wherein the ratio of oxyethylene groups to fatty acid radicals is from 3 to 8.

2. A composition as defined in claim 1 wherein the hexitan partial ester is a sorbitan partial ester.

3. A composition as defined in claim 1 wherein the hexitan partial ester is a mannitan partial ester.

60 4. A yarn carrying a surface coating of a composition as defined in claim 1.

5. A composition comprising (1) from 75 to 98% of a refined mineral oil and (2) from 25 to 2% of a mixture containing (a) from 50 to 20% of a compound of the formula:



wherein R is the residue formed by removal of active hydrogen from a compound of the class consisting of aliphatic alcohols, acids, amines and amides containing from 12 to 18 carbon atoms solely substituted by hydrogen and R<sub>1</sub> is a member of the class consisting of hydroxyl and the residue formed by the removal of active hydrogen from a compound of the class con-

sisting of aliphatic acids and alcohols containing 12 to 18 carbon atoms, solely substituted by hydrogen,  $x$  representing a number from 0 to 9 and  $y$  being an integer less than 3 and (b) from 50 to 80% of a mineral oil soluble material selected from the group consisting of polyoxyethylene ethers of hexitan partial esters of fatty acids having from 12 to 18 carbon atoms wherein the ratio of oxyethylene groups to fatty acid radicals is from 3 to 8, and partial esters of fatty acids having from 12 to 18 carbon atoms with polyoxyethylene ethers of hexitols wherein the ratio of oxyethylene groups to fatty acid radicals is from 3 to 8.

6. A composition as defined in claim 5 wherein R represents an amide and the hexitan partial ester is a sorbitan partial ester.

7. A composition as defined in claim 5 wherein R represents an amine and the hexitan partial esters is a sorbitan partial ester.

8. A composition as defined in claim 5 wherein R represents an aliphatic alcohol and the hexitan partial ester is a sorbitan partial ester.

9. A composition as defined in claim 5 wherein R represents an aliphatic acid and the hexitan partial ester is a sorbitan partial ester.

10. A composition as defined in claim 5 wherein R represents an aliphatic acid and the hexitan partial ester is a mannitan partial ester.

11. A composition comprising (1) 95% of a refined mineral oil and (2) 2.5% of polyoxyethylene stearoyl amide containing 5 oxyethylene groups, and (3) 2.5% of the polyoxyethylene ether of sorbitan tripalmitate containing 16 oxyethylene groups.

12. A composition comprising (1) 80% of refined mineral oil and (2) 5% of polyoxyethylene stearyl amine containing 10 oxyethylene groups and (3) 15% of the polyoxyethylene ether of sorbitan monooleate containing 5 oxyethylene groups.

13. A composition comprising (1) 80% of a refined mineral oil and (2) 5% of polyoxyethylene stearyl alcohol containing 3 oxyethylene groups and (3) 15% of the polyoxyethylene ether of sorbitan monooleate containing 5 oxyethylene groups.

14. A composition comprising (1) 80% of a refined mineral oil and (2) 10% of polyoxyethylene stearic acid containing 7 oxyethylene groups.

groups and (3) 10% of the polyoxyethylene ether of sorbitan monostearate containing 4 oxyethylene groups.

15. A composition comprising (1) 80% of a refined mineral oil and (2) 10% of polyoxyethylene stearic acid stearate containing 10 oxyethylene groups and (3) 10% of the polyoxyethylene ether of mannitan monooleate containing 5 oxyethylene groups.

16. A regenerated cellulose yarn containing as an active surface ingredient a composition comprising a mixture of (1) 80% white mineral oil, (2) 10% of polyoxyethylene stearic acid containing 7 oxyethylene groups and (3) 10% of the polyoxyethylene ether of sorbitan monostearate containing 4 oxyethylene groups.

17. A dyed cotton knitting yarn containing as an active surface ingredient a composition comprising a mixture of (1) 80% of a refined mineral oil and (2) 5% of polyoxyethylene stearyl alcohol containing 3 oxyethylene groups and (3) 15% of the polyoxyethylene ether of sorbitan monooleate containing 5 oxyethylene groups.

18. A scoured wool stock containing as an active surface ingredient a composition comprising a mixture of (1) 80% of refined mineral oil and (2) 5% of polyoxyethylene stearyl amine containing 10 oxyethylene groups and (3) 15% of the polyoxyethylene ether of sorbitan monooleate containing 5 oxyethylene groups.

19. A scoured wool stock containing as an active surface ingredient a composition comprising a mixture of (1) 80% of a refined mineral oil and (2) 10% of polyoxyethylene stearic acid stearate containing 10 oxyethylene groups and (3) 10% of the polyoxyethylene ether of mannitan monooleate containing 5 oxyethylene groups.

#### References Cited in the file of this patent

#### UNITED STATES PATENTS

| Number    | Name           | Date          |
|-----------|----------------|---------------|
| 1,970,573 | Schoeller      | Aug. 21, 1934 |
| 2,380,166 | Griffin        | July 10, 1945 |
| 2,404,240 | MacLaurin      | July 16, 1946 |
| 2,425,755 | Roberts        | Aug. 19, 1947 |
| 2,436,219 | MacLaurin      | Feb. 17, 1948 |
| 2,456,283 | Jefferson      | Dec. 14, 1948 |
| 2,565,403 | Sproule et al. | Aug. 21, 1951 |